

## UNITED STATES PATENT OFFICE

2,411,032

## LUBRICANT

Ernest F. Engelke and William W. Odell, El Dorado, Ark., assignors to Lion Oil Company, a corporation of Delaware

No Drawing. Application January 11, 1944,  
Serial No. 517,840

9 Claims. (Cl. 252—33.6)

1

This invention relates to "an improved lubricant and additive for a lubricant." In particular the invention has to do with the production of a lubricant, particularly a liquid lubricant, which has improved properties through the employment therein of a particular type of material herein-after referred to as an additive; it also has to do with the particular additive so employed. The improvement made in the performance of a lubricant by incorporating therein the herein described additive is characterized particularly by the formation of less gummy and varnish-like deposits inside the piston heads, piston skirts, behind the piston rings, and elsewhere in internal combustion engines, when the lubricant, an oil in this case, with said additive is used as the engine lubricant. The invention is not limited to lubricants which are normally liquid at room temperatures of 60° to 70° F.

Some of the objects of this invention are as follows:

To produce lubricating oils with high detergent characteristics for the prevention of the formation of gummy, varnish-like and carbonaceous materials which normally form with ordinary engine oil and deposit upon the piston skirts, piston heads, and behind the piston rings causing them to be stuck, in internal combustion engines such as Diesel engines after limited periods of operation.

To produce additives with high load carrying capacity.

To produce lubricating oil additives of high wear reducing capacity on the rings, cylinder walls, and bearings of internal combustion engines.

To provide a suitable process by means of which said additives can be produced.

To provide an additive which imparts oxidation inhibiting power to a lubricant when incorporated therein.

Other objects will become manifest from the disclosures made herein.

We have discovered that oil-soluble phosphorus containing soaps, mixed with high molecular-weight alcohols, be these of aliphatic, mixed aliphatic and aromatic, or of purely aromatic or naphthenic nature, when used in proportions of about 1 to 3 percent in a lubricating oil, have the property of controlling the formation and deposition of varnish or lacquer-like materials upon the walls of the pistons, behind the piston rings, and other delicate parts of internal combustion engines when said oil is used as a lubricant therein. The alcohols may be present in the mixture as such

2

or partially or wholly converted into phosphoric acid esters.

We have further discovered that such soaps mixed with high molecular-weight alcohols of the nature described above, tend to suppress to an appreciable extent the oxidation of the oil, thereby preventing the formation, in the oil in use, of acids of a corrosive nature.

We have further discovered that the soaps of certain metals, as for instance silver, tend to deposit an extremely fine layer of metal (plating) on the hottest parts of the engine thereby protecting these against the corrosive attack of organic acids which are in some degree formed inside the motor, especially in motors subjected to severe service.

The starting materials particularly used for the production of the additives forming the subject of this invention are waxes such as bees wax, Chinese wax, carnauba wax, degras, spermaceti, etc. Also liquid waxes such as sperm oil, bottlenose oil and others are suitable. When these waxes are saponified certain high molecular alcohols are formed, such as cetyl, myrisetyl, myristyl and ciryl alcohols, and the cholesterols. Thus, for example, cetyl alcohol may be obtained from spermaceti; myrisetyl alcohol from carnauba wax; cholesterol from degras or wool-fat; and ciryl and myristyl alcohols from beeswax. Japan wax, being a glyceride, is not considered for use in this invention, nor are the so-called animal and vegetable fats, which are, with very few exceptions, esters of low molecular weight polyhydric alcohols, mainly of glycerine.

Also the heavy metal soaps of acids obtained by oxidizing long-chain paraffinic hydrocarbons, as for example paraffine wax, in the liquid phase with air and a suitable catalyst at relatively low temperatures, usually around 160° C., such as for instance those of silver and copper, are suitable particularly when employed in conjunction with a high molecular weight monohydroxy hydrocarbon compound. The oxidation of long chain paraffinic hydrocarbons may be conducted so that besides petroleum acids substantial amounts of high molecular monohydric alcohols are formed; thus a mixture is obtained which may be regarded as identical or at least very similar to a mixture obtained in the saponification of natural waxes.

The preparation of additives according to this invention comprises the following steps. Spermaceti, for example, is saponified in the conventional way with soda lye, yielding a mixture consisting mainly of cetyl alcohol and sodium palmitate. By acidifying the reaction mixture, the

palmitic acid is liberated. The alcohol-acid mixture is carefully washed to remove the last traces of inorganic salts and thereupon the mixture is heated under stirring, for example, in an oil bath to around 300° F. to remove the last traces of moisture. The dry product, chiefly cetyl alcohol and palmitic acid, is then subjected to phosphorization by means of heating and stirring same with 5 percent, based on the weight of the charge, of phosphorus pentoxide, or 2 to 2.5 percent of elemental yellow phosphorus. The temperature of the reaction mass is gradually raised to about 390° F. and kept there 4 to 6 hours. The mass is then allowed to settle at about 200° F. whereby a small amount of sludge usually forms regardless of which of the two agents is used to effect the phosphorization. The clarified or partly clarified supernatent mixture is then passed through a fine-mesh strainer for removing any suspended sludge and then digested at water bath temperature, commonly about 200° F., with the requisite amount of dilute caustic soda lye to bring the palmitic acid into solution. The sodium palmitate is then precipitated with the requisite amount of silver nitrate to convert the sodium palmitate to silver palmitate. The phosphorized mixture of cetyl alcohol and silver palmitate is separated from the mother liquor, thoroughly washed with hot water and dried by heating under agitation at about 280° to 300° F. The product thus obtained is dark colored and it is readily soluble at slightly elevated temperatures in light or heavy motor oils. At room temperature the product is solid. It melts at about 150° to 160° F.

*Example 1*

Use of oil with silver-containing additive. This additive, prepared as described above, of which 0.6 percent was added to a SAE 30 oil was tested under high temperature automotive conditions for 72-hours in a number of Lauson engines. After these tests the engines were found to be in extremely good condition and there was extremely little engine deposit. The piston rings and ring grooves were in excellent condition and the ring wear was very low. When the same SAE 30 oil without the additive was tested in a similar manner in Lauson engines for 72-hours the engines were not in good condition after the run period, and there were considerable engine deposits; some of the piston rings were sticking because of deposits in the ring grooves. Furthermore, the wear and bearing weight loss were appreciably higher when the straight lubricating oil without additives was used in these engine tests. This additive thus possesses both the properties of a detergent and an inhibitor of oxidation.

A 96-hour test of the same oil using the same amount of the same additive therein (0.6 percent) under high temperature automotive conditions (namely, 190° F. cooling water outlet temperature and 285° F. temperature of oil in the pan) gave the following favorable results. Only very slight lacquer formation was in evidence on the pistons and engine parts, not the slightest indication of ring sticking appeared, and the holes in the oil ring were not plugged, which indicates the excellent detergent properties of the additive. The ring weight loss was extremely low and the bearing weight loss was also low. After an extended period of engine operation, the outer sides of the piston rings showed, instead of a carbonaceous deposit commonly found with average engine oil, a slight mirror like deposit of silver.

*Example 2.—Additive preparation*

A commercial grade of neutral degras was saponified in the conventional manner with caustic soda, and the purified and dry saponificate was converted by means of P<sub>2</sub>O<sub>5</sub> in like manner as described in the foregoing example to a phosphorized product, and then converted by means of silver nitrate solution to the silver soap, which was washed and dried in the usual manner. Of this material, including the high molecular weight alcohol formed during saponification, 0.6 percent was incorporated into a SAE 30 grade motor oil and the mixture subjected to a 72-hour test run in Lauson engines under high temperature automotive conditions. The results obtained in this test were the following:

A small amount of lacquer formed on the various parts of the engine but there was not the slightest indication of ring sticking nor of plugging of the oil holes in the rings, which is indicative of a high degree of detergency possessed by the additive under testing. The bearing weight loss was extremely low.

We have found that by similarly using other metals in the place of silver, for example zinc, lube oil additives of a high degree of effectiveness can be produced in a manner analogous to that according to which the silver soap was prepared.

A wax, for example spermaceti, is saponified and phosphorized in the same method by means of which the silver soap was obtained. By precipitation of the aqueous sodium soap solution with a water soluble zinc salt, the zinc soap is obtained in mixture with the other phosphorized constituents of the original material. The precipitated mixture is separated from the mother liquor, washed free of salts, and dried by heating to 300° F. The dried zinc soap product is readily soluble in heavy petroleum oils.

An SAE 30 motor oil doped with 0.6 percent of the above zinc soap and subjected to a 96 hour run in a Lauson motor under high temperature automotive conditions, viz.—190° F. head and 285° F. in the pan with the following results: There was very little lacquer formed on the piston and on the inside of the engine. The piston rings were perfectly clean and free and no trace of plugging of the oil holes in the rings could be detected. This is a strong indication of good detergency of the zinc additive. The bearing weight loss was very low and neither the piston rings nor the cylinder walls showed any loss due to wear.

The additives described in the foregoing were found to be very useful as extreme pressure oil additives as may be understood from a study of the results given below.

The phosphorized mixture composed of mono-atomic alcohols and heavy metal soaps obtained from the various kinds of waxes when subjected to the treatment described in detail in the foregoing showed very considerable film strength enhancing capacity when tested with a Falex film-strength testing machine. An SAE 30 grade motor oil of Mid-Continent origin showed when tested with and without the silver additive the following results:

Blank (average of three tests)—failure at a jaw pressure of 900  
Oil plus 1 percent silver additive, also average of three tests—failure at 2400

which represents a gain of 270 percent in the load-carrying capacity of the doped oil.

Because lacquer deposits in engines is not always due to straight oxidation of the lubricant but frequently to polymerization as well, and because nitric oxide present in engine products of combustion is a catalyst to the formation of lacquers of this type, we have studied these factors and we have found by experiment that the effectiveness of the above described additives is enhanced with respect to reduction of lacquer formation by using them in combination with such materials as phenols, aminophenols and aromatic tertiary amines or combinations of them.

Before defining our claims, attention is called to the fact that the nature of the small amount of carbon deposited on the piston heads of an engine operated with the use of an engine oil employing the above described additives is radically different from that formed when the same oil without the additives is thus employed. The carbon formed, when the above described additives are employed, is soft and can readily be removed from the piston head, whereas when no additive is employed in the lubricating oil the carbon formed is not only much greater in amount but it is hard and adheres to the metal.

In employing aromatic amines we have found it possible to make excellent general purpose mixed additives in which the above described metal soaps are included, for example:

|                                                                  | Percent    |
|------------------------------------------------------------------|------------|
| Silver soap as described                                         | 0.3 to 3.0 |
| Dimethylated aniline of which dimethyl aniline is representative | 0.2 to 0.5 |
| Engine oil sufficient to make 100 percent                        |            |

In place of dimethyl aniline, dipropyl, dibutyl, or diethyl aniline may be used with excellent results. Besides tertiary amines, tertiary butyl and tertiary amyl phenols and their sulphides have been found to be effective when used in small amounts in combination with the soaps described above in retarding the detrimental effect of oxides of nitrogen which are commonly present in the gaseous products of combustion in an internal combustion engine. For example, another general purpose mixed additive oil is as follows:

|                                     | Percent    |
|-------------------------------------|------------|
| Silver additive as described herein | 0.3 to 1.0 |
| Dimethyl aniline                    | 0.2 to 0.9 |
| Tertiary butyl phenol               | 0.3 to 2.0 |

50 Engine oil sufficient to make 100 percent

The examples presented herein are for the purpose of illustrating this invention which is not limited in scope to the specific illustrations.

Having described our invention so that one skilled in the art can practice it, we claim:

1. A lubricant suitable for use in an internal combustion engine, comprising a major proportion of an oil having lubricating characteristics and a minor proportion of an additive sufficient in quantity to prevent oxidation of the lubricant, the sticking of piston rings and the corrosion of bearings, said additive comprising a phosphorized mixture of a soap and a higher molecular monohydric alcohol, said soap being derived from a heavy metal and a member of a group consisting of natural waxes and artificial wax mixtures obtained in the catalytic oxidation of high molecular hydrocarbons of paraffinic crudes, the mixture being phosphorized by the use of a member of a group consisting of elemental phosphorus and phosphorous pentoxide.

2. A lubricant suitable for use in an internal combustion engine, comprising a major propor-

tion of an oil having lubricating characteristics and a minor proportion of an additive sufficient in quantity to prevent oxidation of the lubricant, the sticking of piston rings and the corrosion of bearings, said additive comprising a phosphorized mixture of a soap and a high molecular monohydric alcohol, said soap being derived from a heavy metal and a member of a group consisting of natural waxes and artificial wax mixtures obtained in the catalytic oxidation of high molecular hydrocarbons of paraffinic crudes, the mixture being phosphorized by the use of a member of a group consisting of elemental phosphorus and phosphorous pentoxide, the soap included in the additive being a silver soap.

3. A lubricant suitable for use in an internal combustion engine, comprising a major proportion of an oil having lubricating characteristics and a minor proportion of an additive sufficient in quantity to prevent oxidation of the lubricant, the sticking of piston rings and the corrosion of bearings, said additive comprising a phosphorized mixture of a soap and a high molecular monohydric alcohol, said soap being derived from a heavy metal and a member of a group consisting of natural waxes and artificial wax mixtures obtained in the catalytic oxidation of high molecular hydrocarbons of paraffinic crudes, the mixture being phosphorized by the use of a member of a group consisting of elemental phosphorus and phosphorous pentoxide, the soap included in the additive being a zinc soap.

4. A lubricant suitable for use in an internal combustion engine, comprising a major proportion of an oil having lubricating characteristics and a minor proportion of an additive sufficient in quantity to prevent oxidation of the lubricant, the sticking of piston rings and the corrosion of bearings, said additive comprising a phosphorized mixture of a soap and a high molecular monohydric alcohol, said soap being derived from a heavy metal and a member of a group consisting of natural waxes and artificial wax mixtures obtained in the catalytic oxidation of high molecular hydrocarbons of paraffinic crudes, the mixture being phosphorized by the use of a member of a group consisting of elemental phosphorus and phosphorous pentoxide, the additive including a high molecular monohydric alcohol selected from a group consisting of cetyl, caryl, myrisyl and myristyl alcohols and the cholesterol.

5. A lubricating oil suitable for internal lubrication of internal combustion engines, having high detergent properties comprising principally a petroleum oil having incorporated therein a predetermined amount of a phosphorized mixture of a heavy-metal soap of a wax, said predetermined amount varying from about 0.2 percent to about 2 percent of the whole, according to the amount of beneficiation required by said petroleum oil, said mixture including besides the wax soap the alcohol formed in saponifying the wax.

6. A lubricant suitable for use in an internal combustion engine, comprising a major proportion of an oil having lubricating characteristics and a minor proportion of an additive sufficient in quantity to prevent oxidation of the lubricant, the sticking of piston rings and the corrosion of bearings, said additive comprising a phosphorized mixture of a soap and a high molecular monohydric alcohol, said soap being derived from a heavy metal and a member of a group consisting of natural waxes and artificial wax mixtures obtained in the catalytic oxidation of high molecular hydrocarbons of paraffinic crudes, the mixture

being phosphorized by the use of a member of a group consisting of elemental phosphorus and phosphorous pentoxide, the additive including a small quantity of an organic tertiary amine.

7. A lubricant suitable for use in an internal combustion engine, comprising a major proportion of an oil having lubricating characteristics and a minor proportion of an additive sufficient in quantity to prevent oxidation of the lubricant, the sticking of piston rings and the corrosion of bearings, said additive comprising a phosphorized mixture of a soap and a high molecular monohydric alcohol, said soap being derived from a heavy metal and a member of a group consisting of natural waxes and artificial wax mixtures obtained in the catalytic oxidation of high molecular hydrocarbons of paraffinic crudes, the mixture being phosphorized by the use of a member of a group consisting of elemental phosphorus and phosphorous pentoxide, said additive including a small quantity of a lacquer inhibitor comprising an aromatic tertiary amine.

8. A lubricant suitable for use in an internal combustion engine, comprising a major proportion of an oil having lubricating characteristics and a minor proportion of an additive sufficient in quantity to prevent oxidation of the lubricant, the sticking of piston rings and the corrosion of

5 10 15 20 25

bearings, said additive comprising a phosphorized mixture of a soap and a high molecular monohydric alcohol, said soap being derived from a heavy metal and a member of a group consisting of natural waxes and artificial wax mixtures obtained in the catalytic oxidation of high molecular hydrocarbons of paraffinic crudes, the mixture being phosphorized by the use of a member of a group consisting of elemental phosphorus and phosphorous pentoxide, said additive including a small quantity of a lacquer inhibitor comprising a member of a group consisting of phenols, alkyl phenols, amino phenols and alkyl, aryl and aralkyl substituted sulphides.

9. A lubricating oil adapted for use as a lubricant in internal combustion engines comprising essentially a hydrocarbon oil having incorporated therein approximately 0.3 to 2.0 percent of a phosphorized, heavy metal soap of a wax along with some of the high molecular weight monohydroxy alcohol formed during the saponification of said wax and a small amount of an inhibitor comprising a member of a group consisting of phenols, alkyl phenols, amino phenols and alkyl, aryl and aralkyl substituted sulphides.

ERNEST F. ENGELKE.  
WILLIAM W. ODELL.